

1,357,989.

W. C. JOHNSON,  
ABSORBENT BLOCK,  
APPLICATION FILED MAY 3, 1919.

Patented Nov. 9, 1920.



*William C. Johnson* Inventor

By

*Wood & Wood*

Attorneys

# UNITED STATES PATENT OFFICE.

WILLIAM C. JOHNSON, OF MEMPHIS, TENNESSEE.

## ABSORBENT BLOCK.

1,357,989.

Specification of Letters Patent.

Patented Nov. 9, 1920.

Application filed May 3, 1919. Serial No. 294,537.

To all whom it may concern:

Be it known that I, WILLIAM C. JOHNSON, a citizen of the United States, and residing at Memphis, in the county of Shelby 5 and State of Tennessee, have invented a new and useful Improvement in Absorbent Blocks, of which the following specification is a full disclosure.

My invention deals with the production 10 of a highly absorbent block or pad composed of a cotton fiber or vegetable pulp compressed into a solid unitary body. This product is particularly adaptable as an article of manufacture in the form of a block, 15 inserted within a suitable holder, for use as a blotter, which will quickly and effectively absorb or take up ink, possessing long life and offering many advantages over the ordinary sheet blotter now commonly in use. 20 An object of the invention consists in compressing, by using a simple power or other form of press, a physically and chemically treated wet or moist cotton fiber into a unitary solid mass, and then dried, having 25 substantial density and cohesion and constituting a body characterized by highly absorbent and penetrating properties.

Another object of the invention provides 30 as a new article of manufacture, a cotton fiber compressed into the form of a block or pad for use as a desk blotter.

Other objects and advantages of the same will in part be obvious from the annexed drawings and following description thereof.

35 The drawings illustrate the invention as an article of manufacture preferably in the form of a blotter block inserted within a holder for which the product is particularly adaptable, and in such drawings, like 40 characters of reference denote corresponding parts throughout the several views, of which:

Figure 1 is a plan view of the blotter block and holder.

45 Fig. 2 is a central section through the same.

Fig. 3 is a perspective view of the compressed fiber block.

The fiber stock utilized by my invention 50 comprises a fine cotton fiber or lint which normally adheres to the cotton seed after ginning or to the hulls or capsules, which has to be separated from the hulls or capsules. This fiber or lint is physically and

chemically treated to furnish a clean, purified and bleached stock. 55

The stock which I preferably use, and which has yielded the best results, is the fiber made by the process disclosed in my former Patent No. 530,533, dated Dec. 11, 1894. 60

I have made repeated efforts to find a market for this material, which is produced in great abundance, in mills for making either writing or blotting paper, but so far 65 without encouragement or success.

I have therefore sought to find some useful employment for this material, enabling me to work it up at the mills into a new, useful and distinctive commercial article, 70 and one particularly which will not require the expensive character of machinery and labor essential in paper mills.

It is not necessary, though desirable, to employ a bleached cotton fiber stock, but it 75 is of much greater importance that the stock be subjected to a softening treatment with caustic soda, which does materially soften the stock, and by dissolving out the cellular matter, renders the fibers porous 80 and absorptive to a remarkable degree.

Also, it is not necessary, though highly desirable, to subject these purified fibers to a brushing or beating machine to reduce the knots and kinks and straighten and 85 unify the fiber particles into a more uniform stock which will more completely "pulp" when worked up with water.

I have discovered that when this stock is 90 mixed with water, to about the consistency of buttermilk, the mass can be strained and drained, and compressed into a mold, the fiber giving up its water readily and not tending to flow away with the water.

I have also discovered that when this 95 stock pulp is compressed in a mold, analogous to a brick machine mold, the fibers will felt and interlace into a compact, unitary, brick-like structure, with a uniformly smooth texture, blotting contact under surface, of the nature required in a blotter, and that it has sufficient weight to serve as a blotting paper-weight, and that it has compressibility and permanence of structure adapting it to be interchangeably fitted into a suitable holder. 100

This fiber stock when compressed into a solid unitary mass or block has highly ab-

sorbent and penetrating qualities, which adapts itself to molding into block or brick form for use as a desk blotter and which can be suitably shaped to fit into a holder.

5 The fiber stock after it has been treated under known methods and process to clean the product and while in a wet or pulped condition is compressed into a solid unitary block or pad of any desired thickness, after 10 which it is dried, providing a dense and highly absorbent and relatively ponderous body, thereby successfully converting the stock into a blotting body or block. No expensive or complex machinery is required 15 and a cotton lint or short fiber stock, having high absorbent quality can be converted into a marketable product, and in this form of a block none of the objections obtain 20 which are found when it is attempted to make cotton fiber into a sheet of blotting paper.

Referring to the drawings, 1 indicates the block or pad of cotton fiber compressed or molded to a convenient size and thickness, 25 to fit into a holder 2, interchangeable for a new block after it has been completely saturated with ink. This pad can be made of such thickness that it is almost impossible to so thoroughly saturate it with ink that it 30 will lose its absorbent qualities. With a thick pad it is possible to absorb and take up heavy blots of ink without spreading the same over the surface of the paper.

Further, the absorption is so instantaneous, and fixed, that an ink spot or mark taken up by my device will not restamp upon the writing sheet if accidentally contacting another portion of the sheet immediately after the blotting operation.

40 The cotton-seed-hull fiber preferably is obtainable in almost unlimited quantities for low cost, and my invention so conserves a by-product having substantially no other field of utility at present.

45 The new commodity has also many other useful fields other than as a blotter device, such as table pads, packing, and other uses to which the new article is applicable.

Having described my invention, I claim:

50 1. A new article of manufacture consisting of a mass of absorbent cotton fibers pulped and compressed in a wet state into

a brick, and then dried, constituting a dense, permanent and highly absorbent blotter of a thickness convenient for handling.

55

2. A new article of manufacture consisting of a holder in which is secured a blotter brick formed of a mass of pulped, absorbent fibers, compressed in a wet state and then dried into a dense, unitary structure, the combined holder and blotter brick constituting a combined blotter and paper-weight.

60

3. A new article of manufacture consisting of a mass of highly absorbent cotton fiber, pulped, compressed and molded when wet into a solid, felted brick, and then dried, constituting a durable, homogeneous body adapted for blotting and paper-weight uses, and adapted to be interchangeably used with a suitable holder.

65

4. A new article of manufacture consisting of a mass of highly absorbent cotton fiber, pulped, compressed and molded when wet into a solid, felted brick, and then dried, constituting a durable, homogeneous body characterized by having a smooth, fine texture, bottom-contact surface suitable for blotting writing-paper, adapted for blotting and paper-weight uses, and adapted to be interchangeably used with a suitable holder.

70

5. A new article of manufacture consisting of physically and chemically treated cotton fiber compressed wet and dried into a unitary solid block, constituting a blotter body characterized by highly absorbent, penetrating properties.

75

6. An article of manufacture consisting of purified cotton fibers felted, molded and condensed into a relatively thick, solid and heavy brick, having a smooth, under-surface, adapted to be used as a blotting paper-weight.

80

7. A new article of manufacture consisting of a mass of highly absorbent short cotton fiber or lint, compressed and molded in a wet state into a unitary, solid mass of board thickness, and then dried.

85

In witness whereof, I hereunto subscribe my name, as attested by the two subscribing witnesses.

WILLIAM C. JOHNSON.

Witnesses:

H. S. HAYLEY,  
S. T. ADAMS.

90

95